

## [54] RESISTANCE MATERIAL

[75] Inventors: Alexander H. Boonstra; Cornelis A. H. A. Mutsaers; Franciscus N. G. R. van der Kruis, all of Eindhoven, Netherlands

[73] Assignee: U.S. Philips Corporation, New York, N.Y.

[21] Appl. No.: 74,598

[22] Filed: Sep. 12, 1979

## [30] Foreign Application Priority Data

Sep. 20, 1978 [NL] Netherlands 7809554

[51] Int. Cl.<sup>3</sup> ..... B32B 15/00

[52] U.S. Cl. ..... 338/308; 156/89; 252/518; 428/432; 423/593; 338/309; 428/471; 428/697

[58] Field of Search ..... 428/539, 426, 432, 457, 428/469, 472; 252/518, 521; 427/101-103; 423/593; 156/89; 338/308, 309

## [56]

## References Cited

## U.S. PATENT DOCUMENTS

|           |        |                      |           |
|-----------|--------|----------------------|-----------|
| 3,374,185 | 3/1968 | Nitta et al. ....    | 423/593 X |
| 3,553,109 | 1/1971 | Hoffman ....         | 423/593 X |
| 3,681,262 | 8/1972 | Bouchard ....        | 252/521 X |
| 4,019,168 | 4/1977 | Collins ....         | 428/539 X |
| 4,107,387 | 8/1978 | Boonstra et al. .... | 428/539 X |
| 4,145,470 | 3/1979 | Matsuura ....        | 427/102   |

Primary Examiner—George F. Lesmes

Assistant Examiner—E. Rollins Buffalow

Attorney, Agent, or Firm—Norman N. Spain

## [57]

## ABSTRACT

Resistance material consisting of a mixture of metal oxidic compounds, metal oxides, a permanent binder and a temporary binder, the resistance-determining component consisting of barium-rhodate BaRh<sub>6</sub>O<sub>12</sub>. This component has a linear positive temperature coefficient of the resistance (TCR) and enables the production of a resistor having a very low TCR by combining the material with a material having a negative TCR. The resistor is obtained by firing this resistance material after it has been applied onto a substrate.

5 Claims, No Drawings

## RESISTANCE MATERIAL

The invention relates to a resistance material consisting of a mixture of one or more metal oxides, a permanent and a temporary binder, one or more metal oxides and, possibly, a metal, the material containing a metal-rhodate as the resistance-determining component, and to a resistor consisting of the resistance material providing onto a substrate and from which the temporary binder has been removed by heating and provided with leads.

U.S. Pat. No. 4,107,387 describes such a resistance material in which the resistance-determining component is a metal-rhodate defined by the composition  $M_3Rh_7O_{15}$ , M preferably being Pb or Se.

The advantage of this compound relative to many previously suggested oxides for use as the resistance-determining component in resistance material is that it is a completed-reaction product which, with a permanent binder and, possibly, together with a different resistance-determining component having a different temperature dependency can be assembled in a simple manner on a suitable substrate to form a resistor body. Prior to that resistance pastes were in common usage from which the resistance-determining component was not obtained until firing thereof on a substrate and by reaction with a vitreous binder, for example a lead oxide glass. This required rather long firing times (for example half an hour) at a relatively high temperature (approximately 800° C.).

A further advantage is the linear negative temperature coefficient of the resistance (TCR) of this material, which temperature behaviour is rare. Combining this material with the much commoner material having a linear positive temperature coefficient enables the production of resistors having a very low TCR ( $/TCR/ < 100 \times 10^{-6}/^{\circ}C.$  temperature range—100° to +200° C.).

The invention furnishes a resistance-determining material having a linear positive TCR, also of the rhodate type, which can be assembled together with material having a linear negative TCR into resistors having a low TCR ( $/TCR/ < 100 \times 10^{-6}/^{\circ}C.$ ).

According to the invention the resistance material is characterized in that the resistance-determining component consists of barium rhodate defined by the composition  $BaRh_6O_{12}$ .

Surprisingly, it was found that whereas it was impossible to prepare the barium rhodate in conformity with the composition and the properties stated in the above-mentioned U.S. Pat. No., there is a barium rhodate defined by the composition  $BaRh_6O_{12}$  which has a positive, linear TCR and a totally different crystal structure and an elementary cell of a totally different structure than the known rhodate.

As mentioned above it is possible to assemble resistance bodies having a low TCR value and having a component with a negative linear TCR as the second resistance-determining component.

In accordance with a further elaboration of the invention a metal rhodate  $M_3Rh_7O_{15}$ , wherein M is preferably Pb or Sr in accordance with the above-mentioned U.S.-Specification, is used for the component with the negative linear TCR.

The resistance body is produced with material in accordance with the invention by mixing the resistance-determining component(s) with a permanent binder and an organic temporary binder which can be removed by means of firing. After this mixture has been applied onto a substrate, the temporary binder is volatilized and/or

decomposed by heating, the permanent binder ensuring cohesion by melting, softening or sintering. The permanent binder, is preferably, a low-melting glass but may also be a synthetic resin material.

The invention will now be further explained with reference to the following examples.

Barium-rhodate and lead-rhodate are prepared by heating a mixture of  $BaO$  and  $Rh_2O_3$  in a molar ratio 1:3, and  $PbO$  and  $Rh_2O_3$  in a molar ratio 6:7, respectively, in air for 1 hour at 1000° C. and 3 hours at a temperature of 700° C., respectively, cooling the reaction product out aimed and grinding it to an average grain size of 0.2  $\mu m$ .

Mixtures of these powders are mixed in different ratios with glass powder having an average particle size of 1  $\mu m$  and thereafter processed into a paste by means of benzylbenzoate and ethyl cellulose.

The glass powders employed had the following compositions, expressed in a percentage per weight:

|           | 1    | 2    | 3    |
|-----------|------|------|------|
| $PbO$     | 74.0 | 53.5 | —    |
| $BaO$     | —    | 18.3 | 42.1 |
| $SiO_2$   | 18.6 | 20.2 | —    |
| $B_2O_3$  | 5.0  | 5.4  | 57.9 |
| $Al_2O_3$ | 2.4  | 2.6  | —    |

The pastes are spread on alundum plates which are dried in the air and thereafter fired in air for 15 minutes. The layer obtained is 15  $\mu m$  thick.

The following table shows some mixing ratios and the results obtained therewith. Herein m represents the weight ratio  $BaRh_6O_{12}:Pb_3Rh_7O_{15}$  and n the glass content of the total oxides mixture (without temporary binder) in a percentage by weight.

| glass type | m   | n(wt. %) | R/ $\square$<br>( $k\Omega$ ) | TCR<br>( $10^{-6}/^{\circ}C.$ ) |
|------------|-----|----------|-------------------------------|---------------------------------|
| 1          | 1:1 | 50       | 0.85                          | +80                             |
| 1          | 2:1 | 66       | 1.1                           | +20                             |
| 1          | 5:1 | 80       | 45                            | -70                             |
| 2          | 1:1 | 66       | 0.6                           | 0                               |
| 2          | 2:1 | 75       | 2.2                           | -50                             |
| 2          | 7:1 | 85       | 23                            | +10                             |
| 3          | 5:2 | 50       | 1.2                           | +80                             |
| 3          | 4:1 | 66       | 2.5                           | +20                             |
| 3          | 5:1 | 85       | 310                           | -50                             |

What is claimed is:

1. A resistance material consisting essentially of a mixture of at least one metal oxides compound, a permanent binder and a temporary binder, at least one metal oxide and, as a resistance determining component, a barium-rhodate of the formula  $BaRh_6O_{12}$ .

2. The resistance material of claim 1 wherein in addition there is present a metal rhodate having a negative temperature coefficient of the resistance (TCR) in such a quantity that a desired level of TCR is achieved.

3. A material as claimed in claim 2, characterized in that the component having a negative TCR is a metal-rhodate of the formula  $M_3Rh_7O_{15}$ , where  $M = Pb$  or  $Sr$ .

4. A resistor formed by applying the resistance material of claim 1 to a substrate, heating said resistance material to a temperature sufficiently high to remove said temporary binder and to cause said permanent binder to adhere to said substrate thereby uniting said substrate and said resistance material into a coherent body and providing said coherent body with electrically conductive leads.

5. A novel compound having the formula  $BaRh_6O_{12}$ .

\* \* \* \* \*

UNITED STATES PATENT AND TRADEMARK OFFICE  
CERTIFICATE OF CORRECTION

PATENT NO. : 4,277,542

DATED : July 7, 1981

INVENTOR(S) : ALEXANDER H. BOONSTRA ET AL

It is certified that error appears in the above-identified patent and that said Letters Patent is hereby corrected as shown below:

Claim 3, Line 3, change "where" to --wherein--

Signed and Sealed this

Thirtieth Day of November 1982

[SEAL]

Attest:

*Attesting Officer*

GERALD J. MOSSINGHOFF  
*Commissioner of Patents and Trademarks*